

E. C. WALLACE.  
COMPOSITE PAVEMENT.  
APPLICATION FILED NOV. 23, 1910.

1,115,259.

Patented Oct. 27, 1914.



Witnesses

Virginia Gardner.

Edwin C. Wallace,  
By A. G. DuBois Co  
his Attorneys

# UNITED STATES PATENT OFFICE.

EDWIN C. WALLACE, OF EAST AUBURN, CALIFORNIA.

## COMPOSITE PAVEMENT.

1,115,259.

Specification of Letters Patent. Patented Oct. 27, 1914.

Application filed November 23, 1910. Serial No. 593,860.

To all whom it may concern:

Be it known that I, EDWIN C. WALLACE, citizen of the United States, residing at East Auburn, in the county of Placer and State of California, have invented new and useful Improvements in Composite Pavements, of which the following is a specification.

My present invention has relation to a 10 wearing section of composite pavements; and it contemplates the provision of such a wearing section, adapted to be expeditiously laid at small cost of skilled direction, apparatus, labor and material. The wearing 15 section so constructed combines in a novel way physical properties which it has heretofore been impossible to attain in the wearing section of roadways or pavements.

It has long been recognized in the art, that 20 other things being equal, the softer the bitumen used, and the richer in bituminous content, the greater the durability of the mixture. The softness of the bitumen is determined by traffic conditions. In order to 25 avoid displacement, known as "shifting", "ridging", "waving", or "shoving", it is customary on heavily traveled streets to use bitumen of hard consistency (a #2 needle weighted to 100 grams to penetrate from 30 4-6 millimeters in 5 seconds at 77° E.) While on lighter traffic streets the consistency would be such that the needle would penetrate from 6-8 millimeters under same conditions.

35 By my method of construction I obtain a combined effect. The rigidity of the hard bitumen with the malleability or plasticity of the softer bitumen, and in fact I am enabled to use a softer bitumen than has heretofore been possible. This result is produced in a simple though very effective manner. Instead of preparing the wearing section with a uniform mixture laid in a single coat as is usually done I prepare two dissimilar mixtures and lay in two coats using a 45 hard bitumen for the primary coat by mixing it with a mineral aggregate of relatively coarse particles and spreading this over the foundations to a depth to give required 50 thickness to the completed pavement. Prior to compression I spread over the top of this primary coat a superficial coat of fine mixture prepared with a soft bituminous cementing medium and relatively fine mineral aggregate making the mixture richer in bituminous content than would be practical under

usual method of construction; the spreading of said superficial coat being to a depth of one fourth to five eighths the thickness of the primary coat. After the two coats have been spread as described, compression is applied by means of a roller, tamper or other suitable device. However applied this is the first pressure to which either of the coats have been subjected, and the result is 60 to force the fine soft and rich superficial coat to blend with the harder, coarse and more rigid primary coat at the top of the latter. So effective is the blending and bonding of the two coats that there is no 70 cleavage like joint or line of union between them, but a single layer is produced with a rigid body to resist displacement and a softer more pliable top to resist abrasion.

75 In the drawing, accompanying and hereby made a part hereof: the figure is a vertical sectional view of a portion of a wearing section of a composite pavement produced in accordance with my invention.

The invention alluded to consists in a 80 process of producing a wearing section of a pavement, and for the sake of convenience and brevity I will describe in detail the fabrication of the pavement from which description considered conjunctively with the 85 lettered drawing it will be fully understood.

By reference to the drawing it will appear 90 that A is a prepared foundation which I would emphasize may be of any character consonant with the purpose of my invention.

B is the primary coat of the novel and advantageous wearing section, and C the superficial coat thereof.

95 In the preparation of the primary coat I make use of a mineral aggregate of relatively coarser material which may consist of crushed stone or gravel or a mixture of both combined when deemed expedient with 100 a small proportion of sand or other fine mineral matter. This mineral aggregate is mixed with a relatively hard bituminous cementing medium, (in which a #2 needle weighted to 100 grams will penetrate from 105 4-6 millimeters in 5 seconds at 77 degrees F.) in quantity sufficient to coat all the particles. The primary coat will be spread loosely upon the previously prepared foundation to a depth of 2 inches. Prior to compression of the primary coat herein described a superficial coat of relatively fine 110

mineral matter composed of stone screenings or sand or a mixture of both, all of which will pass a screen of not less than 4 meshes per linear inch combined with a 5 relatively soft bituminous cementing medium (a #2 needle weighted to 100 grams shall penetrate from  $7\frac{1}{2}$  to 25 millimeters in 5 seconds at 77 degrees F.) in quantity sufficient to coat all particles and form an ag- 10 glutinated mass is spread loosely over the top of said primary coat, and compression is then applied as above set forth.

I claim—

15 A pavement consisting of a lower primary layer comprising loosely laid relatively large mineral bodies united by a relatively hard bituminous cement in a manner to afford relatively large fissures between the relatively large mineral bodies, which extend 20 a substantial distance below the uppermost stratum of the primary layer, and an upper secondary layer comprising a homogeneous

mass formed of a relatively soft bituminous cement material mixed with finely divided mineral bodies, the homogeneous mass being 25 applied upon the upper surface of the primary layer, and having integral depending anchor arms thereof compressed into the fissures between the loosely laid relatively large mineral bodies of the primary layer, 30 to extend a substantial distance below the uppermost stratum of the lower layer whereby the homogeneous mass is securely anchored with and upon the primary layer to positively prevent creeping of the homo- 35 geneous mass.

In testimony whereof I have hereunto set my hand in presence of two subscribing witnesses:

EDWIN C. WALLACE.

Witnesses:

A. L. HOUGH,  
VIRGINIA GARDNER.